# EUROPEAN PATENT SPECIFICATION

(11) **EP 2 527 117 B1**
(45) Date of publication and mention of the grant of the patent: **09.11.2016**
(21) Application number: 10844064.5
(22) Date of filing: 23.12.2010
(51) Int. Cl.: B28B 1/093, B28B 1/08

(54) **METHOD AND DEVICE FOR MANUFACTURING ARTIFICIAL STONE**
VERFAHREN UND VORRICHTUNG ZUR HERSTELLUNG EINES KÜNSTLICHEN STEINS
PROCÉDÉ ET DISPOSITIF POUR FABRIQUER DE LA PIERRE ARTIFICIELLE

(30) Priority: 21.01.2010 KR 20100005523
(43) Date of publication of application: 28.11.2012
(73) Proprietor: LG Hausys, Ltd., Seoul 150-721 (KR)
(72) Inventor: KO, Hae-Seung, Cheongju-si Chungcheongbuk-do 361-758 (KR); PARK, Chang-Hwan, Cheongju-si Chungcheongbuk-do 361-745 (KR)
(74) Representative: Winter, Brandl, Fürniss, Hübner, Röss, Kaiser, Polte - Partnerschaft mbB
(86) International application number: PCT/KR2010/009241
(87) International publication number: WO 2011/090268

(56) References cited:
- EP-A1- 0 492 555
- EP-A2- 1 266 734
- WO-A1-97/27982
- WO-A2-2006/122893
- KR-A- 20000 045 850
- KR-A- 20010 045 720
- KR-A- 20080 098 973
- KR-A- 20080 098 973
- KR-B1- 100 274 577
- US-A- 5 280 051
- US-A1- 2007 244 222

## Description

### Technical Field

The present invention relates to a method and device for manufacturing artificial stone, and more particularly to a method and device for manufacturing artificial stone, which maximizes a deposition rate of chips exposed to a surface of artificial stone, thereby achieving more natural expression of an external appearance of the artificial stone while improving resistance against abrasion and staining.

### Background Art

Generally, artificial stone for exterior or interior building materials is produced by mixing various kinds of natural stone chips in a cement base, followed by pressing or simple vibration.

In this case, however, since bubbles are not sufficiently removed from the artificial stone, final products have poor physical properties (strength).

The EP 0 492 555 A1 discloses a composition and a process for the production of artificial marble or granite, wherein a liquid, polymerizable binder and a mineral filler are poured into a mould, the mixture is compacted, optionally under vacuum and optionally by shaking or vibration to eliminate occluded air; the binder is thermally polymerized and finally the obtained slab or block is finished.

A manufacturing method of artificial stones is further described in KR 2008 0098973, the method comprising the mixing of small and large chips of defined size and mixing ratio selected from a resin chip, a native rock chip, and a glass chip, and the use of a vibrator.
WO 97/27982 A1 discloses the preparation cementitious products in form of tiles, slabs or blocks by mixing a granulated stone material and a binding mix comprising cement, water and a plasticizer, spreading the resulting mixture in a mould, subjected it to a first very short deaeration step under the effect of a very high vacuum and to a subsequent vibration step under a lower vacuum, after which the mould goes on to setting and hardening steps.

### Disclosure

### Technical Problem

The present invention is directed to solving such problems of the related art and provides a method and device for manufacturing artificial stone, which maximizes a deposition rate of chips exposed to a surface of artificial stone by mixing two or more kinds of chips in a predetermined ratio and vibrating the mixture in a mold to settle the chips on the bottom of the mold, thereby achieving more natural expression of an external appearance of the artificial stone while improving resistance against abrasion and staining.

### Technical Solution

The above problems are solved according to the present invention by providing a method for manufacturing artificial stone as defined in claim 1 and a device for manufacturing artificial stone as defined in claim 9.

According to a further aspect of the present invention the method for manufacturing artificial stone includes the following modified steps: (c) applying primary vibration to the mold using a vibrator at normal pressure and a vibration rate of 1800 to 7000 revolutions per minute (rpm) for 10 seconds to 1 minute to uniformly disperse the raw material in the mold; (d) evacuating air around the mold for 10 to 30 seconds to create a vacuum of 30 mmHg or more around the mold in order to remove bubbles from the raw material; and (e) applying secondary vibration to the mold using a vibrator at normal pressure and a vibration rate of 1800 to 7000 rpm for 30 seconds to 5 minutes to uniformly disperse the raw material in the mold to mold artificial stone.

According to another aspect of the present invention the device for manufacturing artificial stone is modified by including: a vibrator for primarily vibrating the mold at normal pressure and a vibration rate of 1800 to 7000 rpm for 10 seconds to 1 minute; a vacuum generation unit including a chamber receiving the mold transferred from the primary vibration unit and a vacuum generator capable of evacuating air from the chamber for 10 to 30 seconds to create a vacuum of 30 mmHg or more in the chamber; and a secondary vibration unit including a vibrator for secondarily vibrating the mold transferred from the vacuum generation unit at normal pressure and a vibration rate of 1800 to 7000 rpm for 30 seconds to 5 minutes.

### Advantageous Effects

As such, in a method and device for manufacturing artificial stone according to embodiments of the present invention, two or more kinds of chips are mixed in a predetermined ratio and the mixture is vibrated in a mold to settle the chips on the bottom of the mold to maximize a deposition rate of chips exposed to a surface of artificial stone, thereby achieving more natural expression of an external appearance of the artificial stone while improving resistance against abrasion and staining.

### Description of Drawing

Fig. 1 is a flowchart of a method for manufacturing artificial stone according to one embodiment of the present invention; and
Fig. 2 is a conceptual diagram of a device for manufacturing artificial stone according to one embodiment of the present invention.

### Best Mode

Embodiments of the present invention will now be described in more detail with reference to the accompanying drawings. It should be understood that the accompanying drawings are provided by way of illustration for a more detailed description of the present invention, and do not limit the scope of the invention.

As used herein, the term "artificial stone" includes any cement-based artificial stone or resin-based artificial stone, which can be used as interior building materials or exterior building materials.

Fig. 1 is a flowchart of a method for manufacturing artificial stone according to one embodiment of the present invention.

The method for manufacturing artificial stone according to the embodiment includes: (a) mixing two or more kinds of chips having different grain sizes with a raw material for artificial stone; (b) injecting the raw material mixed with the chips into a mold; and (c) applying primary vibration to the mold using a vibrator at normal pressure and a vibration rate of 1800 to 7000 rpm for 10 seconds to 1 minute to uniformly disperse the raw material in the mold.

Further, the method includes (d) evacuating air around the mold for 10 to 30 seconds to create a vacuum of 30 mmHg or more around the mold in order to remove bubbles from the raw material; and (e) applying secondary vibration to the mold using a vibrator at normal pressure and a vibration rate of 1800 to 7000 rpm for 30 seconds to 5 minutes to uniformly disperse the raw material in the mold to mold artificial stone.

Next, each operation of the method will be described in more detail.

The raw material for artificial stone according to one embodiment may be a resin or a cement slurry.

Here, although any resin used for manufacturing typical artificial stone may be used, the resin according to this embodiment may include at least one selected from the group consisting of, for example, acrylic resins, unsaturated polyester resins, epoxy resins, polyvinyl chloride, polystyrene, polycarbonate, polycarbonate, poly(methyl methacrylate), polyethyleneterephthalate, and styrene-methyl methacrylate copolymers.

Alternatively, the raw material for artificial stone may be a cement slurry, which may include 25 to 35 percent by weight of water based on 100 parts by weight of cement.

If the amount of water in the cement slurry is less than 25 wt%, the cement slurry will undergo deterioration in workability and fluidity, and if the amount of water in the cement slurry exceeds 35 wt%, the final cement product will undergo deterioration in mechanical properties.

The mixing operation (a) may include mixing 125 to 200 parts by weight of chips having a grain size of 3 to 9 mm and 50 to 80 parts by weight of chips having a grain size of 1 to 3 mm based on 100 parts by weight of the raw material.

Here, the raw material for artificial stone may be mixed with two or more kinds of chips having different grain sizes. For example, the chips may include at least one kind of chip selected from the group consisting of resin chips comprising at least one selected from the group consisting of acrylic resins, unsaturated polyester resins, epoxy resins, polyvinyl chloride, polystyrene, polycarbonate, poly(methylmethacrylate), polyethyleneterephthalate, and styrene-methyl methacrylate copolymers; glass chips; colored glass chips; natural stone chips; and colored natural stone chips produced by coloring pulverized natural stone pieces.

In one embodiment wherein the cement slurry is used as the raw material for artificial stone, the cement slurry may be comprised of 170 to 250 parts by weight of natural stone chips having a grain size of 3 to 9 mm, 50 to 100 parts by weight of natural stone chips having a grain size of 1 to 3 mm, 30 to 100 parts by weight of natural stone powder, 25 to 35 parts by weight of water, and 1 to 3 parts by weight of a plasticizer, based on 100 parts by weight of the cement slurry. Here, typical additives known in the art may further be added to the slurry.

Then, the raw material mixed with the chips is injected into a mold and is subjected to primary vibration for 10 seconds to 1 minute to achieve uniform dispersion of the raw material in the mold. If vibration is applied for a period of time less than 10 seconds, it can be difficult to obtain uniform dispersion of the raw material, and if vibration is applied for a period of time exceeding 1 minute, the mixed raw material can be excessively hardened, thereby making it difficult to remove bubbles therefrom.

The raw material for artificial stone mixed with the chips may be spread in a constant thickness within the mold by application of primary vibration, which may be performed at a vibration rate of 1800 to 7000 rpm. If the vibration rate is less than 1800 rprn, it can be difficult to spread the mixed raw material to a uniform thickness within the mold, and if the vibration rate exceeds 7000 rpm, the raw material is likely to escape from the mold during application of primary vibration.

Then, the mold is placed in a typical vacuum chamber, which in turn is evacuated for 10 to 30 seconds to create a vacuum of 30 mmHg or more in the chamber in order to remove bubbles from the raw material.

Then, secondary vibration is applied to the mold using a vibrator for 30 seconds to 5 minutes to mold artificial stone. Here, since chips having a higher specific gravity are settled on the bottom of the mold during application of the secondary vibration, it is possible to increase the amount of chips exposed to a surface of artificial stone, so that the artificial stone produced by the method according to this embodiment has a pleasing external appearance.

Further, in the method for manufacturing artificial stone according to this embodiment, pores formed on the surface of the raw material through which the bubbles are removed from the raw material during the evacuation operation may be filled with the raw material during application of secondary vibration, so that the artificial stone has a dense structure and good mechanical strength.

Finally, the molded artificial stone is sequentially subjected to typical processes, such as curing, releasing and surface grinding, followed by cutting, inspection, and packaging, thereby providing a final product.

Fig. 2 is a conceptual diagram of a device for manufacturing artificial stone according to one embodiment of the present invention.

The device 1 includes a primary vibration unit 10, a vacuum generation unit 20, and a secondary vibration unit 30, and a typical transfer mechanism (for example, a belt conveyer) disposed between the respective units to transfer the mold to the subsequent unit.

The mold is transferred between the respective units and is indicates by different reference numerals 13, 23 and 33 for convenience of description of the mold placed in each of the units.

The primary vibration unit 10 includes a raw material weighing instrument 14 capable of weighing a predetermined amount of a mixed raw material for artificial stone S, a mold 13 into which the weighed raw material S is injected from the weighing instrument 14, and a vibrator 11 for vibrating the mold 13 at normal pressure and a vibration rate of 1800 to 7000 rpm for 10 seconds to 1 minute.

The mold 11 may be supported on a frame 12 or the like during application of vibration, and the frame 12 may be connected to a bottom surface, on which the frame 12 is installed, via an elastic member 15 so as to maintain elasticity upon application of vibration.

The aforementioned operations (a) to (c) of the method may be performed using such a primary vibration unit 10.

The vacuum generation unit 20 includes a chamber 21 which receives the mold 23 transferred from the primary vibration unit 10, and a vacuum generator 24 which is capable of evacuating air from the chamber 21 for 10 to 30 seconds to create a vacuum of 30 mmHg or more in a space 25 of the chamber.

The operation (d) of the method may be performed using such a vacuum generation unit 20.

The secondary vibration unit 30 includes a vibrator 31 for vibrating the mold 33 transferred from the vacuum generation unit 20 at normal pressure and a vibration rate of 1800 to 7000 rpm for 30 seconds to 5 minutes.

Further, the mold 33 may be supported on a frame 32 or the like during application of secondary vibration, and the frame 32 may be connected to a bottom surface, on which the frame 32 is installed, via an elastic member 35 so as to maintain elasticity upon application of vibration.

Each of the units constructed as described above constitutes a single instrument and allows the mold to be transferred therefrom to the next unit after operation corresponding to each unit, thereby enabling continuous operation and mass production.

### Example

Cement-based artificial stone was produced using natural stone chips.

First, a cement slurry acting as a binder for artificial stone was placed in a mold. Here, the cement slurry was comprised of about 150 parts by weight of natural stone chips having a grain size of about 5 mm, about 100 parts by weight of natural stone chips having a grain size of about 2 mm, about 50 parts by weight of natural stone powder, about 30 parts by weight of water, and about 2 parts by weight of a plasticizer, based on 100 parts by weight of the cement slurry.

Then, the cement slurry was placed in the mold and subjected to primary vibration for about 15 seconds using a vibrator to spread the cement slurry to a constant thickness within the mold, which in turn was placed in a vacuum chamber. Then, the vacuum chamber was evacuated for about 25 seconds to create a vacuum within the chamber in order to remove bubbles from the cement slurry. Then, the mold was subjected to secondary vibration for about 3 minutes using a vibrator to maximize the deposition rate of the chips by settling the natural chips on the bottom of the mold, followed by curing the cement slurry for 12 hours at 40 to 50°C under constant moisture conditions.

After curing the cement slurry, the cured product was released from the mold and subjected to typical grinding and cutting processes for artificial stone to provide 400 mm(L)x400 mm(W)x20 mm(T) artificial stone.

### Comparative Example

Artificial stone according to the comparative example was produced by the same method as that of the example except that the vacuum generating operation was not performed.

Bending strength and absorption rate of the artificial stone products according to the example and the comparative example were measured, and results are shown in Table 1.

**Table 1**

| | Example | Comparative Example |
|---|---|---|
| Bending strength (N/mm²) | 13.5 | 11.2 |
| Absorption rate (%) | 1.5 | 2.5 |

As can be seen from Table 1, the artificial stone according to the example has high bending strength and a low absorption rate.

## Claims

1. A method for manufacturing artificial stone, comprising:
(a) mixing two or more kinds of chips having different grain sizes with a raw material (S) for artificial stone;
(b) injecting the raw material (S) mixed with the chips into a mold (13, 23, 33);
(c) applying primary vibration to the mold (13) using a vibrator (11) at normal pressure to uniformly disperse the raw material (S) in the mold (13);
(d) evacuating air around the mold (23) to create a vacuum around the mold (23) in order to remove bubbles from the raw material (S);
(e) applying secondary vibration to the mold (33) using a vibrator (31) at normal pressure to mold artificial stone;
(f) curing and demolding the molded artificial stone;
(g) surface-processing of the artificial stone; and
(h) cutting, inspection, and packaging of the artificial stone.

2. The method of claim 1, wherein the raw material (S) is a resin or a cement slurry.

3. The method of claim 2, wherein the resin comprises at least one selected from the group consisting of acrylic resins, unsaturated polyester resins, epoxy resins, polyvinyl chloride, polystyrene, polycarbonate, poly(methyl methacrylate), polyethyleneterephthalate, and styrene-methyl methacrylate copolymers.

4. The method of claim 2, wherein the cement slurry contains 25 to 35 parts by weight of water based on 100 parts by weight of cement.

5. The method of claim 1, wherein the mixing of two or more kinds of chips comprises mixing 125 to 200 parts by weight of chips having a grain size of 3 to 9 mm and 50 to 80 parts by weight of chips having a grain size of 1 to 3 mm based on 100 parts by weight of the raw material (S) for artificial stone.

6. The method of claim 1, wherein the chips comprise at least one kind of chip selected from the group consisting of resin chips, glass chips, colored glass chips, natural stone chips, and colored natural stone chips produced by coloring pulverized natural stone pieces.

7. The method of claim 1, wherein the primary vibration and the secondary vibration are applied at normal pressure and a vibration rate of 1800 to 7000 rpm.

8. The method of claim 1, wherein the evacuation is performed to create a vacuum of 30 mmHg or more.

9. A device for manufacturing artificial stone, comprising:
a primary vibration unit (10) including a raw material (S) weighing instrument (14) capable of weighing a predetermined amount of a mixed raw material (S) for artificial stone, a mold (13, 23, 33) into which the weighed raw material (S) is injected from the weighing instrument (14), and a vibrator (11) at normal pressure for primarily vibrating the mold (13);
a vacuum generation unit (20) including a chamber (21) receiving the mold (23) transferred from the primary vibration unit (10) and a vacuum generator (24) capable of evacuating air from the chamber (21) to create a vacuum in the chamber (21); and
a secondary vibration unit (30) including a vibrator (31) at normal pressure for secondarily vibrating the mold (33) transferred from the vacuum generation unit.

10. The device of claim 9, wherein primary vibration and secondary vibration are applied at normal pressure and a vibration rate of 1800 to 7000 rpm.

11. The device of claim 9, wherein the vacuum generator evacuates air from the chamber to create a vacuum of 30 mmHg or more in the chamber.

12. The device of claim 9, wherein the raw material (S) is a resin or a cement slurry.

13. The device of claim 12, wherein the resin comprises at least one selected from the group consisting of acrylic resins, unsaturated polyester resins, epoxy resins, polyvinyl chloride, polystyrene, polycarbonate, poly(methyl methacrylate), polyethyleneterephthalate, and styrene-methyl methacrylate copolymers.

14. The device of claim 12, wherein the cement slurry contains 25 to 35 parts by weight of water based on 100 parts by weight of cement.

## Patentansprüche

1. Verfahren zur Herstellung eines künstlichen Steins, umfassend:
(a) Mischen von zwei oder mehreren Arten an Splittern mit unterschiedlichen Korngrößen mit einem Rohmaterial (S) für einen künstlichen Stein;
(b) Einspeisen des mit den Splittern vermischten Rohmaterials (S) in eine Form (13, 23, 33);
(c) Anwenden einer ersten Vibration auf die Form (13) unter Verwenden eines Vibrators (11) bei Normaldruck, um das Rohmaterial (S) in der Form (13) gleichmäßig zu verteilen;
(d) Abpumpen von Luft um der Form (23) herum zum Erzeugen eines Vakuums um die Form (23) herum, um Blasen aus dem Rohmaterial (S) zu entfernen;
(e) Anwenden einer zweiten Vibration auf die Form (33) unter Verwenden eines Vibrators (31) bei Normaldruck, um einen künstlichen Stein zu formen;
(f) Aushärten und Entformen des geformten künstlichen Steins;
(g) Oberflächenbearbeiten des künstlichen Steins; und
(h) Schneiden, Überprüfen und Verpacken des künstlichen Steins.

2. Verfahren nach Anspruch 1, wobei das Rohmaterial (S) ein Harz oder ein Zementbrei ist.

3. Verfahren nach Anspruch 2, wobei das Harz mindestens eines umfasst ausgewählt aus der Gruppe bestehend aus Acrylharzen, ungesättigten Polyesterharzen, Epoxyharzen, Polyvinylchlorid, Polystyrol, Polycarbonat, Poly(methylmethacrylat), Polyethylenterephthalat und Styrol-Methylmethacrylat-Copolymeren.

4. Verfahren nach Anspruch 2, wobei der Zementbrei 25 bis 35 Gewichtsteile an Wasser bezogen auf 100 Gewichtsteilen an Zement enthält.

5. Verfahren nach Anspruch 1, wobei das Mischen der zwei oder mehreren Arten an Splittern ein Mischen von 125 bis 200 Gewichtsteilen an Splittern mit einer Korngröße von 3 bis 9 mm und 50 bis 80 Gewichtsteilen an Splittern mit einer Korngröße von 1 bis 3 mm bezogen auf 100 Gewichtsteile des Rohmaterials (S) für einen künstlichen Stein umfasst.

6. Verfahren nach Anspruch 1, wobei die Splitter mindestens eine Art an Splittern umfasst ausgewählt aus der Gruppe bestehend aus Harzsplittern, Glassplittern, farbigen Glassplittern, Natursteinsplittern und farbigen Natursteinsplittern, die hergestellt werden durch Färben von pulverisierten Natursteinstücken.

7. Verfahren nach Anspruch 1, wobei die erste Vibration und die zweite Vibration bei Normaldruck und einer Vibrationsrate von 1800 bis 7000 Upm angewendet werden.

8. Verfahren nach Anspruch 1, wobei das Abpumpen durchgeführt wird, um ein Vakuum von 30 mmHg oder mehr zu erzeugen.

9. Vorrichtung zur Herstellung eines künstlichen Steins, umfassend:
eine erste Vibrationseinheit (10) mit einer Wiegeeinrichtung (14) für das Rohmaterial (S), die in der Lage ist eine vorbestimmte Menge eines gemischten Rohmaterials (S) für einen künstlichen Stein abzuwiegen, einer Form (13, 23, 33) in welche das abgewogene Rohmaterial (S) von der Wiegeeinrichtung (14) eingespeist wird und einem Vibrator (11) bei Normaldruck zum ersten Vibrieren der Form (13);
eine Vakuumerzeugungseinheit (20) mit einer Kammer (21) zur Aufnahme der von der ersten Vibrationseinheit (10) weitergeleiteten Form (23) und einem Vakuumgenerator (24) der in der Lage ist, Luft aus der Kammer (21) abzupumpen, um in der Kammer (21) ein Vakuum zu erzeugen; und
eine zweite Vibrationseinheit (30) mit einem Vibrator (31) bei Normaldruck zum zweiten Vibrieren der von der Vakuumerzeugungseinheit weitergeleiteten Form (33).

10. Vorrichtung nach Anspruch 9, wobei die erste Vibration und die zweite Vibration bei Normaldruck und einer Vibrationsrate von 1800 bis 7000 Upm angewendet werden.

11. Vorrichtung nach Anspruch 9, wobei der Vakuumgenerator Luft aus der Kammer abpumpt, um in der Kammer ein Vakuum von 30 mmHg oder mehr zu erzeugen.

12. Vorrichtung nach Anspruch 9, wobei das Rohmaterial (S) ein Harz oder ein Zementbrei ist.

13. Vorrichtung nach Anspruch 12, wobei das Harz mindestens eines umfasst ausgewählt aus der Gruppe bestehend aus Acrylharzen, ungesättigten Polyesterharzen, Epoxyharzen, Polyvinylchlorid, Polystyrol, Polycarbonat, Poly(methylmethacrylat), Polyethylenterephthalat und Styrol-Methylmethacrylat-Copolymeren.

14. Vorrichtung nach Anspruch 12, wobei der Zementbrei 25 bis 35 Gewichtsteile an Wasser bezogen auf 100 Gewichtsteile an Zement enthält.

## Revendications

1. Procédé pour la fabrication d'une pierre artificielle, comprenant :
(a) le mélange de deux types ou plus de fragments ayant des granulométries différentes avec une matière première (S) pour la pierre artificielle ;
(b) l'injection de matière première (S) mélangée avec les fragments dans un moule (13, 23, 33) ;
(c) l'application d'une vibration primaire au moule (13) en utilisant un vibreur (11) à une pression normale pour disperser uniformément la matière première (S) dans le moule (13) ;
(d) l'évacuation de l'air autour du moule (23) pour créer un vide autour du moule (23) afin d'éliminer les bulles de la matière première (S) ;
(e) l'application d'une vibration secondaire au moule (33) en utilisant un vibreur (31) à une pression normale pour mouler une pierre artificielle ;
(f) le durcissement et le démoulage de la pierre artificielle moulée ;
(g) le traitement de surface de la pierre artificielle ; et
(h) la découpe, l'inspection et l'emballage de la pierre artificielle.

2. Procédé selon la revendication 1, dans lequel la matière première (S) est une résine ou une pâte de ciment.

3. Procédé selon la revendication 2, dans lequel la résine comprend au moins un élément sélectionné dans le groupe constitué de résines acryliques, de résines de polyester insaturé, de résines époxy, de chlorure de polyvinyle, de polystyrène, de polycarbonate, de poly(méthyl-méthacrylate), de polyéthylène-téréphtalate, et de copolymères styrène-méthyl-méthacrylate.

4. Procédé selon la revendication 2, dans lequel la pâte de ciment contient 25 à 35 parties en poids d'eau sur la base de 100 parties en poids de ciment.

5. Procédé selon la revendication 1, dans lequel le mélange de deux types ou plus de fragments comprend le mélange de 125 à 200 parties en poids de fragments ayant une granulométrie de 3 à 9 mm et 50 à 80 parties en poids de fragments ayant une granulométrie de 1 à 3 mm, sur la base de 100 parties en poids de matière première (S) pour une pierre artificielle.

6. Procédé selon la revendication 1, dans lequel les fragments comprennent au moins un type de fragment choisi dans le groupe constitué de fragments de résine, de fragments de verre, de fragments de verre coloré, de fragments de pierre naturelle, et de fragments de pierre naturelle colorée produits en colorant des morceaux de pierre naturelle pulvérisés.

7. Procédé selon la revendication 1, dans lequel la vibration primaire et la vibration secondaire sont appliquées à une pression normale et à une vitesse de vibration de 1 800 à 7 000 tr/min.

8. Procédé selon la revendication 1, dans lequel l'évacuation est réalisée pour créer un vide de 30 mmHg ou plus.

9. Dispositif de fabrication d'une pierre artificielle, comprenant :
une unité de vibration primaire (10) comprenant un instrument de pesée (14) de la matière première (S) capable de peser une quantité prédéterminée d'une matière première mélangée (S) pour une pierre artificielle, un moule (13, 23, 33), dans lequel la matière première pesée (S) est injectée depuis l'instrument de pesée (14) et un vibreur (11) à une pression normale pour faire vibrer de manière primaire le moule (13) ;
une unité de génération de vide (20) comprenant une chambre (21) recevant le moule (23) transféré de l'unité de vibration primaire (10) et un générateur de vide (24) capable d'évacuer l'air de la chambre (21) pour créer un vide dans la chambre (21) ; et
une unité de vibration secondaire (30) comprenant un vibreur (31) à une pression normale pour faire vibrer de manière secondaire le moule (33) transféré depuis l'unité de génération de vide.

10. Dispositif selon la revendication 9, dans lequel la vibration primaire et la vibration secondaire sont appliquées à une pression normale et à une vitesse de vibration de 1 800 à 7 000 tr/min.

11. Dispositif selon la revendication 9, dans lequel le générateur de vide évacue l'air de la chambre pour créer un vide de 30 mmHg ou plus dans la chambre.

12. Dispositif selon la revendication 9, dans lequel la matière première (S) est une résine ou une pâte de ciment.

13. Dispositif selon la revendication 12, dans lequel la résine comprend au moins un élément choisi dans le groupe constitué de résines acryliques, de résines de polyester insaturées, de résines époxy, de chlorure de polyvinyle, de polystyrène, de polycarbonate, de poly(méthyl-méthacrylate), de polyéthylène-téréphtalate, et de copolymères de styrène-méthyl-méthacrylate.

14. Dispositif selon la revendication 12, dans lequel la pâte de ciment contient 25 à 35 parties en poids d'eau sur la base de 100 parties en poids de ciment.
